

Patented Dec. 10, 1929

1,739,475

# UNITED STATES PATENT OFFICE

HENDRIK JAN JAKOB JANSSEN, OF ARNHEM, NETHERLANDS, ASSIGNOR TO NAAM-  
LOOZE VENNOOTSCHAP NEDERLANDSCHE KUNSTZIJDEFABRIEK, OF ARNHEM,  
NETHERLANDS

## PROCESS OF MANUFACTURING DYED ARTIFICIAL SILK

No Drawing. Application filed December 15, 1925, Serial No. 75,620, and in Germany December 15, 1924.

My invention relates to a process for altering artificial silk and the like with respect to its absorptive power for dyes. It is known, in weaving artificial silk on looms of the 5 Jacquard type, to dye the silk with different dyes and to weave this silk on the looms in patterns.

I have found, however, that it is possible to work the artificial silk on looms of the Jacquard type in an undyed condition and to obtain color effects in dyeing the piece goods. This I attain by using artificial silk with different absorptive power for dyes and in such a way that I treat an amount of material 15 with a certain absorptive power so that part of it obtains a larger or smaller absorptive power than the other part of the batch.

It is a known art to prepare artificial silk with a larger or smaller absorptive power for 20 dyes by ripening the viscose longer or shorter.

My invention aims, however, at affecting the absorptive power for dyes of prepared artificial silk in quite another way, namely by altering the contents of non-cellulosic substances, such as oxy cellulose, hemicellulose, 25 hydrocellulose, by means of suitable measures.

For instance, my process may be carried out in such a way that the contents of oxy cellulose of the fibres and in consequence 30 thereof the absorptive power for dyes is increased by heating the fibres or threads in air or in oxidizing means.

If the absorptive power for dyes is required to be decreased I may treat the prepared threads with substances which remove the oxy cellulose, hemicellulose or hydrocellulose wholly or partially. I have obtained favorable results in heating the prepared threads in glycerine and subsequently washing the 35 thus treated material. However, I may also use other materials than glycerine, provided that they do not unfavorably affect the artificial silk.

The following examples are merely illustrative and in no way are to be understood as limiting the scope of my patent.

### Example 1

Ordinary viscose silk prepared in any of 40 the known ways is heated in glycerine at ap-

proximately 150° C. Then the artificial silk is washed and dried in the usual way. Thereupon the silk is dyed in a watery solution of methylene blue containing about half a gram of dye per liter, at a temperature of about 55 80° C. It will appear that the silk is colored a light blue and that the same viscose silk not treated with heated glycerine will have after being treated in the same dye of the same concentration and temperature a dark blue color. 60

If the silk is treated at room temperature with a diluted solution of sodium hypochlorite during two hours the same will after washing and drying obtain a darker color than non-treated silk. 65

### Example 2

Ordinary viscose silk is heated with glycerine in the way as specified in Example 1. After washing and drying the same is dyed 70 in a bath containing about 1 gram of diamond fuchsin per liter. It appears that the threads obtain a bright red color, which is much lighter than that obtained by untreated artificial silk. 75

Having thus described my invention, what I claim as new and desire to secure by Letters Patent is:—

1. The process of modifying the dye absorptive properties of artificial silk containing oxy cellulose, hemicellulose or hydrocellulose which comprises treating said silk with glycerine in a heated state. 80

2. The process of modifying the dye absorption properties of artificial silk made from 85 viscose containing oxy cellulose, hemicellulose or hydrocellulose, which comprises treating it with heated glycerine.

In testimony whereof I affix my signature.

HENDRIK JAN JAKOB JANSSEN

90

95

100